

## UNITED STATES PATENT OFFICE

2,115,161

## HAIR WAVING COMPOUND AND PROCESS

Ernest O. Frederics, Bronxville, and James C. Brown, Mount Vernon, N. Y.; said Brown as signor to said Frederics

No Drawing. Application March 16, 1934.  
Serial No. 715,916

10 Claims. (Cl. 167—87.1)

This invention relates to compounds and methods used in the permanent waving of human hair. It has for a primary object the production of an improved compound and the development of new 5 operating conditions by which an exceptionally tight wave may be imparted in a brief time to all types of hair. The invention is particularly effective for the waving of thin, fine hair which is always the most difficult to deal with.

10 In the permanent waving of human hair, tufts or groups of strands are ordinarily coiled more or less tightly about metal rods and are then surrounded with pads of absorbent material which have previously been saturated with a solution 15 of some special compound. The pads usually have metal foils attached which when wrapped around the tufts of hair provide reasonably tight encasements. Each tuft of hair as so prepared is then inserted in a suitable heater, or other device, 20 in which the temperature may be raised to, say, 100° C. and maintained for a suitable period of time.

Solutions of various characters have been suggested for use in saturating the pads. In the 25 pending application of James C. Brown, Ser. No. 656,147, filed February 10, 1933, there is disclosed the advantage of using any of a number of organic amines under specified conditions either alone or in combination with ammonia. Now, 30 we have discovered that exceptional results may be obtained by the employment of a solution containing three or more distinct amino compounds having successively higher boiling points. For example, a solution containing a low boiling 35 amine, (such as ethylamine) ammonia, and a higher boiling amine (such as diethylamine) has been found to give most excellent results. Apparently as a solution of this character is brought to a temperature of between 75° and 100° C., the 40 ethylamine is first volatilized most rapidly; then as the temperature rises and a large part of this constituent has been vaporized, the ammonia is set free in greater quantities and finally the diethylamine is more largely vaporized. Therefore, 45 in a treatment extending over a period of, say, 10 minutes, active vapors of first one and then another of the amino compounds will be more or less constantly liberated. It will be understood, of course, that a certain amount of 50 each of the compounds will be volatilized at all times, or until completely driven off, but as the temperature rises, the higher boiling constituents will come into greater prominence. In this way effective action of the vapors throughout the 55 treating period is insured with the result that the time of the treatment may be reduced.

In using the mixture of three amino compounds, as suggested above, it will ordinarily be found most satisfactory to use substantially equal 60 amounts of the three ingredients, or the am-

monia may predominate to a certain extent. The quantity of the various ingredients used may vary according to the character of hair being treated and other considerations, such as the nature of the process being employed. It has been found 5 that from 1 to 10 grams of each of the compounds, diethylamine, ethylamine, and ammonia, added to sufficient water to produce 100 grams of solution, will form a very satisfactory hair waving 10 solution under practically all conditions and for all types of hair. Ordinarily it will be found that from 2 to 5 grams of each of the constituents in sufficient water to make up 100 grams of solution will be most satisfactory. As explained in the 15 above mentioned application, it is desirable that the solution, when utilized at ordinary atmospheric pressure, should have a pH value of not less than 11.6 and not higher than 12.2. Sufficient water should be added at all times to keep the pH value below the higher limit specified. 20 Furthermore, to be effective, the water content should be low enough not to produce a pH value below 11.6. While, as stated above, it is considered preferable to employ substantially equal 25 amounts of the three amino compounds, this may be varied to suit particular circumstances so that one ingredient may be used in two or three times greater proportion than another. In fact each 30 ingredient may be varied between the limits previously specified, i. e., 1 gram to 10 grams in 100 grams of solution, independently of the other ingredients.

As already indicated, the strength of the solution employed should vary somewhat with the character of the hair being treated. For example, 35 fine, thin hair, which is difficult to provide with a wave, should ordinarily be treated with a stronger solution, i. e., one having a higher pH value than coarser or heavier hair. We have also discovered that the pH value desired in the conduct of the process may be varied considerably by the development of pressure around the coiled tufts of hair. For example, if a vapor pressure of .5 pound is created and maintained within the 40 foil or similar enclosure for the hair, the pH value of the solution may, and preferably should, be dropped to between 10 and 10.5. If a higher vapor pressure is employed, the pH value may and should be reduced even further. For example, 45 if a pressure of 2 pounds is employed, the pH value of the solution may be as low as 9 and preferably should not be a great deal higher. For a vapor pressure of 5 pounds above atmospheric, a pH value of 8 is quite satisfactory. If a pressure as high as 15 pounds above atmospheric were maintained around the coiled hair, 50 the permanent wave could be imparted with steam alone. It would not be necessary to add the ammonia or any of the amino or other alkaline compounds. Ordinarily the difficulty of main- 55

taining a steam-tight jacket capable of withstanding 15 pounds pressure around the hair and the danger of having steam at this pressure escape near the scalp of the person being treated 5 will prevent the use of such a high pressure. On the other hand, a pressure of between .5 and 2 pounds, or even up to 5 pounds, above atmospheric may very readily be employed with the result that a much weaker solution will be sufficient 10 to impart a permanent wave to the hair within the time ordinarily required for treatment of this character, or if the strength of the solution is maintained, the time may be reduced.

While the three specified amino compounds, 15 i. e., ethylamine, diethylamine and ammonia, have been found to be particularly effective for the production of a tight and permanent wave, in a relatively short period of time, other combinations of three or more amino compounds may also 20 be employed to advantage. It will ordinarily be desirable to employ ammonia as one of the ingredients and it has been found that ethylamine is more effective than any other compound as a second ingredient of the mixture. However, 25 the diethylamine, and even the ethylamine, may be replaced by other amines and particularly by aliphatic amines containing from 2 to 6 carbon atoms. For example, such compounds as propyl or butyl amines and piperazine may be substituted 30 for one or both of the amines specified in the preferred solution.

As a specific example of a highly satisfactory composition for the waving of an average type of hair, 2 grams of each of the ingredients, ethylamine, diethylamine and ammonia, may be added to 94 grams of water or to a similar quantity of a solution prepared in accordance with Letters Patent No. 1,637,469 or 1,681,170. Other specific mixtures which will be found superior to waving 10 compounds previously employed may contain the following:

|              | Grams |
|--------------|-------|
| Ethylamine   | 3     |
| Ammonia      | 5     |
| Diethylamine | 2     |
| Water        | 90    |
| Ethylamine   | 1.5   |
| Ammonia      | 5     |
| Diethylamine | 1.5   |
| Water        | 92    |

In employing a solution of the type contemplated by the present invention, the temperature need not and preferably should not be raised to the boiling point of water. A temperature of, say, 80° C. or between 70° and 90° C. will ordinarily be found quite effective, particularly if the solution used has a relatively high pH value. When a weaker solution is employed, and especially if the pressure around the hair is raised to a point above atmospheric, a somewhat higher temperature will ordinarily be required or found desirable. When the treatment is carried out under pressure, this may be established either by 65 the vaporization of the solution and the confinement of the vapors or in any other convenient way, as by the direct introduction of steam or vapors, generated at any point, into the enclosure around the hair.

70 While the preferred and other illustrative forms of the invention have been disclosed in considerable detail, it will be understood that various changes may be made in the nature and quantity of the ingredients employed and in the conditions

under which the treatment is carried out without departing from the general spirit and scope of the invention. Although a water solution is preferred, it will be understood that the amino compounds may be incorporated in the pads directly 5 or may be distributed over or through the absorbent pads in other ways.

What we claim is:

1. A hair waving composition comprising a solution in water of at least three compounds of the group consisting of aliphatic amino compounds containing two to six carbon atoms and ammonia, each of said compounds having different boiling points all below 100° C. 15

2. A hair waving composition comprising a solution in water of at least three compounds of the group consisting of aliphatic amino compounds containing two to six carbon atoms and ammonia, each of said compounds having boiling points all below 100° C. and spaced more than 10° C. apart. 20

3. A hair waving composition comprising a solution in water of ammonia, ethylamine and another aliphatic amine containing two to six carbon atoms of higher boiling point than ethylamine but below 100° C. 25

4. A hair waving composition comprising a solution in water of ammonia, ethylamine and diethylamine.

5. A hair waving composition comprising a solution in water of ammonia, ethylamine and diethylamine in sufficient quantity to produce a pH value of between 11.6 and 12.2. 30

6. A hair waving composition comprising a solution in water of ammonia, ethylamine and diethylamine, each of said ingredients being present 35 in the proportion of 1 to 10 grams in sufficient water to produce 100 grams of solution.

7. A method of imparting a permanent wave to human hair which comprises subjecting the hair while coiled about a rod to the successive action 40 of the vapors of a plurality of different compounds of the group consisting of aliphatic amino compounds containing two to six carbon atoms and ammonia, each of said compounds having different boiling points during a single treatment. 45

8. A method of imparting a permanent wave to human hair which comprises subjecting the hair while coiled about a rod to the action of the vapors of a plurality of different compounds of the group consisting of aliphatic amino compounds containing 2 to 6 carbon atoms and ammonia, the vapors of the several compounds being successively liberated in greater proportions during the period of treatment from a solution containing all of said compounds. 50

9. A method of imparting a permanent wave to human hair which comprises winding a tuft of hair about a rod, wrapping the hair so coiled in an absorbent pad saturated with a solution of ammonia, ethylamine and diethylamine having a pH 60 value of between 11.6 and 12.2, and applying heat to vaporize the constituents.

10. A method of imparting a permanent wave to human hair which comprises winding a tuft of hair about a rod, wrapping the hair so coiled in an absorbent pad saturated with a solution of ammonia, ethylamine and diethylamine having a pH value of between 8 and 10.5, applying heat to vaporize the constituents, and confining the vapors so formed to establish a super-atmospheric pressure between .5 and 5 pounds around the hair. 70

ERNEST O. FREDERICKS.  
JAMES C. BROWN.